

# UNITED STATES PATENT OFFICE.

ARCHIBALD CLAUDE EVANS, OF HAMPTON WICK, AND PERCY JOSE MITCHELL, OF  
WESTMINSTER, LONDON, ENGLAND.

## METHOD OF MANUFACTURING FINELY-DIVIDED CARBON AND BY-PRODUCTS FROM COAL-PITCH.

1,175,732.

Specification of Letters Patent. Patented Mar. 14, 1916.

No Drawing.

Application filed December 22, 1915. Serial No. 68,248.

To all whom it may concern:

Be it known that we, ARCHIBALD CLAUDE EVANS and PERCY JOSE MITCHELL, residing at Lucerne House, Hampton Wick, Middlesex, England, and Caxton House, Westminster, London, S. W., England, respectively, have invented certain new and useful Improvements in the Method of Manufacturing Finely-Divided Carbon and By-Products from Coal-Pitch; and we do hereby declare the following to be a full, clear, and exact description of the invention, such as will enable others skilled in the art to which it appertains to make and use the same.

This invention relates to an improved method for the manufacture of carbon powder, that is to say, a finely comminuted material which is allied to lamp black but which by reason of its manufacture cannot be technically described as such.

Heretofore in treating coal pitch for the manufacture of carbon powder by means of naphtha it has not been possible to employ the same naphtha over and over again without purification because of the presence of phenols and sulfur compounds which as a feature of applicants' process are removed by the previous treatment of the coal pitch with an alkaline solution. Moreover by avoiding a complete removal of said prior alkaline washings as a further feature of the invention a frothing necessarily occurs which offers considerable advantage when the introduction of the naphtha is made.

Having in mind the state of facts as set out above, the objects of our invention are to provide a convenient and economical process for the production of carbon powder and valuable by-products from pitch.

A further object of our invention is to provide a process for obtaining the products above mentioned in which the solvent may be employed over and over again without purification.

The invention is carried out as follows:— Crude coal pitch is heated to a temperature of about 100 degrees centigrade in a closed still or other suitable vessel. It is then mixed with a weak solution of caustic soda, caustic potash or other suitable basic oxids or hydroxids and agitated for the purpose of removing the phenols and any sulfur

compounds that may be present. The alkaline solution used is preferably of about one-eighth per cent. strength, and the amount used per charge of pitch is equal by weight to that of the pitch. The mixture is then allowed to stand, when the aqueous solution rises to the top and may be removed by a siphon or other convenient means. One method which may with advantage be adopted for this purpose is to leave a small layer of alkaline solution at the top of the pitch and then to add a considerable quantity of cold water. In this way a crust is formed on the surface of the pitch which facilitates the process of siphoning. It is important that a certain amount of moisture or aqueous solution should be left in the pitch for reasons which will be described hereafter.

The next stage of the process is to dissolve out the oils and other constituents of the pitch and leave the free carbon behind. For this purpose ordinary commercial solvent naphtha is used. The treatment with naphtha is preferably carried out in the same vessel as that which is used for the alkali treatment. A quantity of naphtha equal to three times the weight of the pitch used is added to the latter which is warmed to a temperature of 100° centigrade, and violently agitated, the said temperature being maintained throughout the operation. In order to facilitate the solvent action of the naphtha it is important that the pitch on being heated should froth or separate into a large number of small particles, and this end is best achieved by allowing a certain amount of water to remain in the pitch from the previously described alkaline washing. The amount of moisture necessary for this purpose is not large but it is difficult to state a definite quantity; the same can however be easily determined by a trial experiment. If this precaution be ignored it will be found that the pitch will have a tendency to ball or separate into lumps, and the solvent action of the naphtha will thus be greatly impeded, the completion of this part of the process thus requiring considerably longer time and heating than is the case if the precaution referred to above is taken. By these means a

- fairly thick solution is obtained, and to this a second portion of solvent is added cold, the contents of the still being kept at 100° centigrade and agitated for a few minutes.
- 5 This second portion of naphtha may be either once or twice the amount in weight of the pitch used according as it is desired to, obtain perfectly pure carbon or carbon containing a small amount of bitumen.
- 10 The still is preferably fitted with a reflux condenser of any known and suitable type. If desired this second naphtha treatment as a further feature of the invention may be carried out under pressure in which case
- 15 the still used for the whole process may be of any known type of pressure heating apparatus, the initial naphtha treatment being carried out under atmospheric pressure. The mixture is now allowed to stand, when
- 20 the carbon, or most of it, will settle to the bottom as a sludge, while the liquid will separate into one or more layers which can be run off or decanted by suitable draw-off cocks, siphons or other suitable means.
- 25 If desired a filter press may be used at any stage after this second naphtha treatment in order to accelerate the separation of the carbon.
- The carbon is obtained in a finely divided
- 30 but usually rather crude state, and it will generally require re-washing with naphtha, in which case the settling, filtration and decantation processes may be repeated as before. As regard the quantities of naphtha
- 35 used for this and the other washings referred to, it should be stated that excepting in the case in which the highest degree of purity in the carbon may be required, the total amount of naphtha used in the process
- 40 need not exceed six times the weight of pitch. As has been stated, three times the weight of pitch in naphtha are used for the first treatment, once or twice the weight of pitch is used for the second treatment,
- 45 and the amount used for this final washing is regulated by the amount previously used in such a way that the total weight used does not exceed six times that of the pitch. After final decantation of the liquids or
- 50 separation therefrom of the carbon by any suitable means the latter is dried in a closed vessel and heated to drive off any volatile residues which may if desired be collected by suitable condensers. The carbon is thus
- 55 obtained in a finely divided caked condition, and it may then be removed from the vessel, disintegrated or ground in any suitable appliance, and finely pulverized pure carbon obtained.
- 60 As regards the quantities of naphtha used in the processes, it should be stated that six times the weight of pitch in naphtha will suffice to produce what may be regarded as a fairly pure carbon. For certain purposes it has been found desirable for the

carbon to contain a small quantity of bitumen thus facilitating the molding of the powder into any desired shape, and the quantity of bitumen left in the product may be regulated as described by the amount of naphtha used for the second and third washings. If the very highest degree of purity in the carbon is required it may be that the total amount of washing naphtha may exceed six times the weight of pitch, and any desired number of washings with naphtha may be imparted to the carbon without departing from the spirit of the invention.

After the naphtha washings have been freed, either by settling and decantation, or by the use of a filter press, from all traces of free carbon, they are distilled for the purpose of recovering the solvent oils and other substances held in solution. In this recovery process any convenient method of fractional distillation may be used and the process will yield, firstly, the solvent, secondly any intermediate oils contained in the pitch and thirdly a pitch absolutely free from all acid substances and from all free carbon. If necessary the products obtained in the recovery process, both solvent and oils, can be re-distilled for the purpose of purification, and any convenient known type of fractionating column or the like can be used for such purification.

It will thus be seen that this process yields at will either an absolutely pure carbon in a finely divided state or a carbon containing a small quantity of bitumen which renders it suitable for certain special purposes, and in addition that valuable by-products from the pitch are recovered. Apart from the working losses which cannot be avoided in any manufacturing process there is no loss of solvent, which latter can be used over and over again, and similarly the phenols and sulfur compounds removed in the preliminary alkaline treatment may if desired be recovered by any suitable means while the alkaline solution may be used for a number of charges of pitch without being renewed.

We claim:—

1. A method of manufacturing finely divided carbon consisting in first treating coal pitch in a hot condition with a weak alkaline solution, substantially removing the washings and subsequently digesting the mass with solvent naphtha, then separating the free carbon by allowing the mass to settle and decanting or drawing off the liquors with or without the assistance of a filter press.
- 115
2. A method of manufacturing finely divided carbon consisting in first treating coal pitch in a hot condition with a weak alkaline solution, substantially removing the washings from the pitch but leaving a small
- 120
- 125
- 130

quantity of moisture or alkaline solution therein, heating the mass to cause frothing, digesting the mass with solvent naphtha, and then separating the free carbon.

5 3. A method of manufacturing finely divided carbon and by-products consisting in first treating coal pitch in a hot condition with a weak alkaline solution, substantially removing the washings and subsequently digesting the mass with solvent naphtha, sepa-

rating the free carbon, and distilling the remaining liquid for a by-product.

In testimony whereof we affix our signatures in presence of two witnesses.

ARCHIBALD CLAUDE EVANS.  
PERCY JOSE MITCHELL.

Witnesses:

FRANK B. DEHM,  
H. C. WESTON.